

## UNITED STATES PATENT OFFICE

2,121,755

## PROCESS FOR MAKING PATTERNED EFFECTS ON CREPE FABRICS AND PRODUCTS THEREFROM

George Heberlein, Jun., Wattwil, Switzerland,  
assignor to Heberlein Patent Corporation, New  
York, N. Y., a corporation of New York

No Drawing. Application June 19, 1934, Serial  
No. 731,391. In Germany June 22, 1933

9 Claims. (Cl. 26—69)

This invention relates to a process for producing patterned effects on crepe fabrics and to patterned fabrics obtained thereby. In the copending application Serial No. 716,430, filed March 19, 1934, which has now issued as Patent No. 2,035,946, there is described a process for the production of patterned effects on crepe fabrics, according to which a crepe fabric is treated with a parchmentizing agent at some time prior to its final shrinkage to produce a pattern design and then the so treated fabric is treated by a creping bath. This resulted in a crepe fabric having a crepe background with translucent pattern portions thereon, or vice versa.

15 The crepe fabric referred to in said copending application is usually made by weaving yarns, all or a part of which are highly twisted, and then subjecting these yarns to hot soap, caustic solution or other bath to produce the well-known curly or crimped effect characteristic of crepe.

The principal object of the present invention is to provide a process for producing similar patterned effects on crepe fabric in a different manner.

25 The invention comprises the novel products as well as the novel processes and steps of processes according to which such products are manufactured, the specific embodiments of which are described hereinafter by way of example and in accordance with which we now prefer to practice the invention.

It has now been found in accordance with the present invention that patterned effects on crepe fabrics can be produced by treating a crepe fabric at some time prior to its final shrinkage with a binder to produce a pattern design capable of resisting the subsequent wet treatment to which such fabrics are subjected, such as creping and bleaching baths. Then upon subjecting the fabric to a creping treatment, the portions of the fabric untreated with the binder produce the crepe effect, and the portions treated with the binder do not crepe appreciably. The effect of the binder is to render these portions more translucent than the crepe portions under ordinary conditions. The preferred binder is an animal protein substance, such as albumin, animal glue or gelatin. This material is preferably applied in a water solution and is thereafter made water insoluble and resistant to the wet treatments of the creping process by treatment with a hardening agent, such as by coagulation by heating, or tanning as by chromium salts, aluminum compounds, formaldehyde and formaldehyde compounds. Instead of the insolubilized substances

just mentioned, there may be also employed natural or artificial prepared resin suitable for resisting the operations of the creping process above mentioned and there may also be employed cellulose esters and cellulose regenerated from viscose or copper-oxide-ammonium solutions.

5 The fabrics employed according to this invention may be grey (rohe), as well as pretreated fabrics. In the case of the pretreated fabrics which are the most important in commercial use, these fabrics are treated in a manner similar to that described in the above mentioned application Ser. No. 716,430. That is, the previously shrunk fabric in crepe condition, which has a preliminary crepe effect, is stretched to 10 the original grey width and then treated with the binding material and then finally creped. Because of the different dyeing properties of the portions treated with the reserve or binder as compared with the untreated portions, various 15 dyed color effects can be obtained. In addition dyestuffs can be added to the binder before printing. On the other hand, where a dyed fabric is to be treated, a discharge may be added to 20 the binder to be printed thereon. Besides yarns 25 of vegetable fiber such as cotton and linen, the various artificial silks of regenerated cellulose and animal fibers, for instance highly twisted fine wool and silk yarns, may be subjected to 30 the process.

The following are examples of the process employing the steps in the manner in which it is now preferred to practice the invention. These examples are purely illustrative and are not to be construed in a limiting sense.

35 Example 1

A georgette fabric of viscose silk containing highly twisted threads as it comes from the loom ready to be subjected to treatment to produce the 40 crepe effect, is printed in a pattern with a 10% water solution of gelatin heated to 45° C. The printed fabric is then dried. Thereafter the fabric is passed through a 2% formaldehyde solution and is dried at as high a temperature as 45 possible without injury to the material. After this treatment, the printed fabric is subjected to a crepe effecting treatment, as by placing it in a hot soap bath at about 80° C. in the usual manner for creping, and a crepe effect is produced. 50 Thereupon the portions untreated with the insolubilized gelatin binder will crepe, while the portions treated with the insolubilized gelatin binder will remain substantially uncreped. Thereafter, if the fabric treated is held loose 55

while drying, the shrunk creped portions of the fabric will cause the binder treated portions to become somewhat puffed with wave-like elevations and corresponding hollows. The portions treated with the insolubilized gelatin will also appear more translucent and will be stiffer than the untreated portions. The material produced is a crepe fabric having a patterned effect thereon made up of a crepe background with a translucent somewhat stiff design thereon or vice versa, the translucent portion containing insolubilized binder.

*Example 2*

15 As mentioned above, fabrics which are already in crepe condition may also be employed to produce new patterned effects. A cotton fabric for creping is bleached in the usual manner. Great shrinking thereby takes place and the crepe effect is produced on the fabric. While the fabric is drying and still in moist state, it is put under tension along its width and length so that it assumes substantially its original size before creping. It is then printed with an 8% acetyl cellulose solution and dried. Thereafter the fabric so treated is passed through a hot soap creping-bath, from which it is removed and dried without tension. The effect produced is similar to that given in Example 1 above.

20 30 While the invention has been described in detail according to the preferred manner of carrying out the process, it will be obvious to those skilled in the art after understanding the invention, that changes and modifications may be made therein without departing from the spirit or scope of the invention, and it is intended in the appended claims to cover all such changes and modifications.

35

What is claimed as new and desired to be secured by Letters Patent is:

40 1. A process for producing patterned effects on crepe fabrics, which comprises treating a crepe fabric containing highly twisted yarn which will shrink in the creping operation, at 45 some time prior to its final shrinkage, to provide areas which are covered with a substantially insoluble binder, which areas are capable of resisting wet treatments of the usual creping operation, and then subjecting the fabric to 50 creping treatment, causing the portions of the fabric untreated with the binder to crepe, and leaving the treated portions substantially un-

creped and permanently covered with the substantially insoluble binder.

2. A process for producing patterned effects on crepe fabrics, which comprises applying a crepe fabric at some time prior to its final shrinkage with a binder consisting of an animal protein such as gelatin to produce a pattern design, insolubilizing the pattern design so that it will resist wet treatment of the usual creping operation, and then subjecting the fabric to a 10 creping treatment and thereby causing the portions of the fabric untreated with the binder to crepe, leaving the treated portions still containing the binder substantially uncreped.

15 3. A crepe fabric having a patterned effect thereon made up of a crepe background having shrunk highly twisted threads with a translucent somewhat stiff design thereon, the translucent portion containing unshrunk highly twisted threads and a binder.

20 4. A crepe fabric having a patterned effect thereon made up of a crepe design having shrunk highly twisted threads therein with a translucent somewhat stiff background with the translucent background containing unshrunk highly twisted threads and a binder.

25 5. A process according to claim 2 in which the gelatin is insolubilized by treatment with formaldehyde.

30 6. A process for producing patterned effects on crepe fabrics which comprises applying to a crepe fabric at sometime prior to its final shrinkage a binder which is soluble to some extent in the ordinary shrinking bath for the crepe effect thereby forming a pattern on the fabric, insolubilizing the pattern design so that it will resist the action of said bath, and then subjecting the fabric to a creping treatment and thereby causing the portions of the fabric untreated with the binder to crepe, leaving the treated portion 40 substantially uncreped and permanently covered with the substantially insoluble binder.

35 7. A process according to claim 1, in which the binder is a resin.

45 8. A crepe fabric having a crepe area and a stiffened area, the stiffened area containing unshrunk, highly twisted threads and a water-insoluble binder.

50 9. A process according to claim 1, in which the binder is applied as a solution of a cellulose ester from which the solvent is then evaporated.

GEORGE HEBERLEIN, JUN.